

## UNITED STATES PATENT OFFICE

JONATHAN NEWTON WHITE, OF NEW YORK, N. Y.

## ALLOY

No Drawing.

Application filed November 12, 1929. Serial No. 406,722.

This invention relates to an alloy of copper, zinc and manganese in such proportions as to provide a high degree of ductility and resistance to crystallization and fatigue.

Metals and alloys of various kinds are commonly employed in the construction of tubes, strips, diaphragms, bellows and the like, in situations requiring a certain amount of flexibility. One example of such use is in 10 the thermostatic apparatus where there is a movement required for opening and closing valves, and the metal or alloy is formed into bellows, or corrugated or coiled so as to expand and contract with changes in temperature. Another example of such use is in apparatus conveying liquids, gases, vapors, etc., such as oil to bearings or movable parts, gasoline to tanks or mixture receptacles, steam or oil to moving parts, and air or gas 15 to molding apparatus. Many other uses which necessitate a connection that is flexible or semi-flexible are familiar to those skilled in this art. In all such cases it is of great importance to construct such parts of 20 a metal or alloy which has to a high degree the property of resisting crystallization and fatigue under the conditions of operation.

The alloy which forms the subject matter of the present invention is intended primarily for use in apparatus such as above described, but it will of course be obvious that its utility is in no sense restricted to this particular field. The alloy contains a high percentage of copper with smaller percentages 25 of zinc and manganese, as essential components, the copper representing at least 88%, the manganese  $\frac{1}{2}$  to 4%, and the balance zinc.

A particularly favorable composition for 30 the manufacture of corrugated tubing contains 93 to 95% copper, 1 to  $1\frac{1}{4}$ % manganese, and the balance zinc. This mixture or composition showed decided superiority and uniformity of results when subjected to vibratory tests in comparison with commercial brass compositions.

These compositions in accordance with the 35 invention are of good mechanical strength, offer a high degree of ductility and resistance to crystallization and fatigue, and are

readily obtained substantially free from porosity.

It will be understood that inert impurities or additions which do not injuriously affect the good qualities of the alloy composition 55 may be present in association with the copper, manganese and zinc, which are the essential components by which the properties of the alloy are determined.

I claim:

1. An alloy comprising at least 88% copper,  $\frac{1}{2}$  to 4% manganese, and the balance zinc.
2. An alloy comprising 93 to 95% copper, 1 to  $1\frac{1}{4}$ % manganese, and the balance zinc.

J. NEWTON WHITE.

60

65

66

70

75

80

85

90

95

100